

## UNITED STATES PATENT OFFICE

FREDERICK F. MCINTOSH, OF GLEN OSBORNE, PENNSYLVANIA, ASSIGNOR TO CRUCIBLE STEEL COMPANY OF AMERICA, A CORPORATION OF NEW JERSEY

## ALLOY STEEL

No Drawing.

Application filed January 12, 1928. Serial No. 246,384.

This invention has to do with the class of steel now generally called stainless steel, and including the lower-carbon variety which has the arbitrary trade-name of stainless iron. 5 It is a well known fact that the difficulty of machining all of the standard grades of this class of steel has prohibited its use for many industrial purposes. As the result of an 10 extended experimental investigation I have found that by increasing the percentage of some of the elements necessarily present in the steel, but heretofore considered undesirable and therefore kept below definite maximum limits, a stainless steel can be produced which is, relatively speaking, freely 15 machinable, while at the same time it retains, for practical purposes, its distinguishing property of surface stability.

Stainless steel is primarily distinguished 20 in composition by its high percentage of chromium content, not less than eight per cent, and it may contain minor percentages of other alloying elements. Its carbon content should not exceed one per cent. See 25 United States Letters Patent No. 1,197,256 and No. 1,299,404. Commercial products now on the market range in carbon content from about 0.10 per cent to 0.50 per cent and in chromium from about eleven per cent to 30 eighteen per cent, or even more. Small percentages of manganese, not more than 0.50 per cent, are usually present, while the unavoidable contents of sulphur and phosphorus are strictly limited to not more than 35 0.03 per cent of each. As above stated, steel within the above composition ranges is difficult to machine. For example, in rifling a .30 caliber gun-barrel made of the most suitable commercial grade of stainless steel 40 it has been possible to turn out only about one barrel per hour with about thirty grinds on the tool.

I have discovered that by materially increasing the contents of manganese, sulphur 45 and phosphorus, respectively, in the standard grades of stainless steel, a steel will be obtained which is, comparatively speaking, freely machinable. For example, in rifling .30 caliber gun-barrels made of my improved 50 stainless steel more than two barrels per hour

have been turned out, with only one grind on the tool per barrel.

In the lower ranges of carbon content my improved stainless steel contains, approximately, carbon, 0.10-0.20 per cent, manganese, 0.90-1.30 per cent, phosphorus, 0.08-0.15 per cent, sulphur, 0.05-0.15 per cent, silicon, 0.25-0.50 per cent, and chromium, 11-15 per cent. A very desirable composition within the above limits is, carbon, 0.15 per cent, manganese, 1.02 per cent, phosphorus 0.093 per cent, sulphur, 0.107 per cent, silicon, 0.38 per cent, and chromium, 12.21 per cent. This steel was quenched in oil from 1850° F. and drawn back to 1125° F. Its Brinell hardness then was 286, its tensile strength was 129,150 pounds per square inch, its yield point was 112,050 pounds, its elongation in two inches was 19.5 per cent, and its reduction in area 52 per cent. The same steel was 70 subjected to carefully standardized drilling tests in comparison with several commercial grades of so-called stainless iron (carbon, 10-12, chromium, 11-14). Under the same standard conditions the stainless iron could 75 be drilled only about 2 inches, while the drilling of my improved stainless averaged 7.44 inches.

In order to give the best machinable qualities it is recommended that the steel shall be 80 hardened and tempered to give it a Brinell hardness of from 265 to 290, although for particular purposes it can be made either softer or harder.

I use the term stainless steel in the sense 85 that it has come to be used in the art of ferrometallurgy, as denoting a type of alloy steel, usually within the field defined in the two Letters Patent above mentioned (either or both), although in some case a particular 90 product may in one respect or another lie somewhat outside that field and still possess the same essential qualities. It is also well recognized that all grades and specific compositions of stainless steel will not be equally 95 resistant to surface deterioration by the same agencies or under the same conditions; on the other hand, one composition or grade will be the better suited for one purpose and another for another. Therefore I use the 100

term as covering a class of steel having high surface stability, and having carbon and chromium contents within the limits first above set forth and as more generally stated in the said two Letters Patent, and especially in the Letters Patent No. 1,299,404.

I claim as my invention:

- 10 1. Alloy steel containing from about 0.10 per cent to about 1 per cent of carbon, from about 8 per cent to about 18 per cent of chromium, from about 0.9 per cent to about 1.3 per cent of manganese, from about 0.08 per cent to about 0.15 per cent of phosphorus, and from about 0.05 per cent to about 0.15 per cent of sulphur.
- 15 2. Alloy steel containing from about 0.10 per cent to about 0.20 per cent of carbon, from about 11 per cent to about 15 per cent of chromium, from about 0.9 per cent to about 1.3 per cent of manganese, from about 0.08 per cent to about 0.15 per cent of phosphorus, and from about 0.05 per cent to about 0.15 per cent of sulphur.

In testimony whereof I have hereunto set  
25 my hand.

FREDERICK F. McINTOSH.

30

35

40

45

50

55

60

65